

July 15, 1930.

A. W. BURWELL

1,770,876

ARTIFICIAL SHELLAC AND PROCESS OF MAKING THE SAME

Original Filed Dec. 20, 1926



*Inventor*  
Arthur W. Burwell

*By Byrnes Townsend & Bruckenstein*  
*his Attorney*

## UNITED STATES PATENT OFFICE

ARTHUR W. BURWELL, OF NIAGARA FALLS, NEW YORK, ASSIGNOR TO ALOX CHEMICAL CORPORATION, OF NEW YORK, N. Y., A CORPORATION OF NEW YORK

## ARTIFICIAL SHELLAC AND PROCESS OF MAKING THE SAME

Original application filed December 20, 1926, Serial No. 156,052, and in Great Britain October 6, 1927. Divided and this application filed January 12, 1928. Serial No. 246,096.

This invention relates to shellac-like products having many of the characteristics of natural shellac, to a process of making the same, and to compositions containing these products.

I have found that, by the liquid-phase oxidation, under controlled conditions, of hydrocarbons or mixtures thereof such as those occurring in petroleum oils, there may be obtained a variety of oxidation products including formic acid, light ketones and aldehydes, heavy ketones and aldehydes, water-insoluble carboxylic acids which are soluble in the hydrocarbon mixture, and water-insoluble hydroxy-carboxylic acids which are insoluble in the hydrocarbon mixture.

An object of the present invention is to provide petroleum hydrocarbon oxidation products which consist essentially of saponifiable, water-insoluble hydroxy-carboxylic acids insoluble in petroleum hydrocarbon mixtures. More specifically, the present invention concerns the shellac-like products obtained by the controlled oxidation of mid continent or Pennsylvania petroleum distillates having a density of from about 40° to about 36° Baumé, i. e., the so-called fuel oil distillates, although I have found that these products are obtainable from other petroleum distillates than those just mentioned, such as, for example the distillates having a density of 33° to 18° Baumé.

The process of making these shellac-like products consists generally in the liquid-phase oxidation of hydrocarbons or mixtures thereof, under such conditions as to promote the formation of saponifiable, water-insoluble, petroleum-insoluble hydroxy-carboxylic acids and the isolation of the said acids from the partially oxidized mass.

Although this invention is not restricted to the use of any particular hydrocarbon or mixture of hydrocarbons, I prefer to use as starting material the lowest cost petroleum distillate obtainable. For example, the so-called

fuel oil distillate having a density of 40°-36° Baumé, has been found to be advantageous due to its relatively low cost. In general, it may be stated that the proneness to form petroleum-insoluble hydroxy-carboxylic acids is particularly inherent in those petroleum hydrocarbon mixtures which are of relatively higher specific gravity and which contain a minimum of crystallizable bodies (e. g. wax).

The invention will be described and illustrated hereinafter by reference to a batch process, it being understood, however, that the procedure may be made continuous, as shall be explained.

In the accompanying drawing there is shown diagrammatically one form of apparatus suitable for use in carrying out the process of the invention.

The oxidation step proper takes place in an upright cylindrical reaction vessel or oxidizer 1, which may be, for example, about 5 feet in diameter and about 16 to 18 feet in height. The oxidizer 1 may be made of any suitable material such as iron or steel and should be capable of withstanding pressures up to 350 pounds per square inch. Preferably, the oxidizer 1 should be made of or lined with material which is resistant to the corrosive action of the reaction mixture; for example, provided with an inner shell of aluminum 2. The oxidizer is provided at a point near its lower end with a tight coil 3 which serves as a heating or cooling coil as required. Suitable means, not illustrated, such as a jacket surrounding the oxidizer, also may be used to control the temperature of the oxidation reaction. At a point between the lower end of the oxidizer 1 and the tight coil 3 is an air spray pipe 4 connected by pipe line 5 to an air compressor 6. Air spray pipe 4 is so

designed that air is ejected from it in the form of fine bubbles. 7, 8 and 9 are valved hydrocarbon supply pipe, a valved liquid discharge pipe and a valved gas discharge pipe, respectively. 10 is a pressure gauge, and 11 is a

thermometer. 12 is a separating tank fed by the valved liquid discharge pipe 8 leading from the oxidizer 1; said tank being provided with agitating means (not shown).

5 From the bottom of the separating tank 12 extend the valved conduits 13 and 14 for the transference of fluids to the still 17 and to the acid water tank 21 respectively. 16 is a valved supply pipe for conducting water to the separating tank 12. 18 is a condenser, 19 is a distillate receiver and 20 is a vacuum pump. 22 is a valved conduit for admitting air, steam, or the like, to the still 17. 23 is a valved conduit for the transference of distillate from the distillate receiver 19 to the valved conduit 14'. 24 is a swing suction or decantation device in separating tank 12.

The process is carried out in the apparatus illustrated as follows:

20 A petroleum hydrocarbon mixture, such as, for example, the 40°-36° Baumé fuel oil distillate above mentioned, is charged into the oxidizer 1, a small amount of an oxidizing catalyst or exciter of oxidation, such as 25 a compound of manganese copper or iron,—say manganese oleate,—amounting to about 0.1 percent of the weight of the oil is added and the mixture heated up to a temperature in the neighborhood of 120° C. or higher, 30 preferably to about 135-140° C., and an oxidizing gas, preferably air, is supplied through the spray pipe 4. Gases are permitted to accumulate in the oxidizer until the desired pressure is reached, after which 35 the pressure is maintained or regulated by controlling the discharge of gases through the valved gas discharge pipe 9. The pressure may vary considerably, say from 150 to 350 pounds per square inch. The preferred 40 pressure will depend upon a number of conditions, including the temperature maintained, the kind of hydrocarbon mixture under treatment, the rate of air supply and, if oxygen-enriched air is used, upon the richness 45 of the oxygen supply. It is preferred to carry out the oxidation process under such conditions that the reaction is substantially self-sustaining. In general, the reaction is self-sustaining at a temperature of about 50 135°-140° C., and at a pressure of about 250 pounds per square inch, with the hydrocarbon under treatment, although temperatures and pressures may vary between wide limits. Thus, for example, oxidation has been observed at a temperature as low as 100° C.; it is more rapid above 120° C., and the temperature may be allowed to rise to 155° C. with satisfactory results under some circumstances. Therefore, while I prefer to carry 55 out the oxidation process at a temperature at which the reaction rate is fairly rapid, say 135°-140° C., it is to be understood that the invention includes the employment of all suitable temperatures at which oxidation 60 takes place.

During the oxidizing treatment, as is stated above, gases collecting in the upper end of oxidizer 1 are released through the pipe 9. These gases contain practically no oxygen, but do contain carbon dioxide, nitrogen and varying quantities of volatile acids, ketones and other products of the oxidation. The volatile acids, ketones and other products may be condensed in a suitable condenser (not shown) and further treated for the recovery of formic acid, mixed light ketones, etc.

70 During the course of the treatment of the petroleum distillate in the oxidizer 1, there appear to be formed, during the earliest stages of oxidation, formic acid and high molecular weight ketonic and/or aldehydic bodies; continued oxidation results in the production of saponifiable water-insoluble carboxylic acids having molecular weights 75 approximately one and one-half times those which would naturally be calculated for acids derived from the original (i. e., unoxidized) hydrocarbons. Prolonged oxidation converts these petroleum-soluble carboxylic acids into petroleum-insoluble hydroxy-carboxylic acids having about the same, or lower, molecular weights as those which would naturally be calculated for acids derived from the original hydrocarbons, low 80 molecular weight ketonic and/or aldehydic bodies, water, and additional amounts of 85 formic acid.

85 For the purposes of the invention, it is desirable to continue the oxidation treatment 90 until the maximum amount of the petroleum-insoluble hydroxy-carboxylic acids has been obtained while avoiding undue decomposition of the hydrocarbons, as evidenced by an excessive amount of carbon dioxide in the 95 effluent gases and vapors passing to the condenser through the valved gas discharge pipe 9. Usually this occurs when the mass in the oxidizer 1 contains from 25-35% of petroleum-insoluble matter. At this point, which 100 may be determined either by observing a sample of the mass from the oxidizer, by titration, or by observations as to the time and rate of flow of the air for a given quantity of starting material and the undue increase in the relative amount of carbon dioxide in the effluent gases, the reaction mixture in the oxidizer 1 is discharged through the 105 valved liquid discharge pipe 8 into the separating tank 12.

110 Upon settling, the reaction mixture separates into three layers. The bottom layer is found to consist of a strongly acid, aqueous solution of water-soluble acids together with some unsaponifiable matter which is soluble 115 in this strong solution. This layer is drawn off, through the valved conduit 14, into the acid water tank 21. The intermediate layer consists essentially of hydroxy-carboxylic acids which are insoluble in the reaction mix- 120

70

75

80

85

90

95

100

105

110

115

120

125

130

ture, and the top layer is found to be a mixture comprising unoxidized petroleum, petroleum-soluble carboxylic acids, some hydroxy-carboxylic acids, and primary oxidation products, such as, for example, ketonic and/or aldehydic compounds, primary and secondary alcohols, ethers, and possibly some esters.

After the settling has proceeded to the point where the supernatant oil is perfectly clear, the said top layer carefully is withdrawn by means of the swing suction 24, transferred through the valved conduit 14' to the petroleum distillate supply tank 15, and there mixed with fresh distillate in the preferred proportions of 2:1 for use in charging the oxidizer for a subsequent oxidation treatment. Said mixture, consisting of fresh distillate and material which has already been subjected to oxidation treatment, does not require the presence of an oxidizing catalyst or exciter of oxidation to effect normal oxidation, the reaction proceeding in a manner identical to that observable upon oxidizing a fresh charge of the distillate containing the added exciter of oxidation.

The residue in the separating tank 12, comprising saponifiable, petroleum-insoluble, water-insoluble, hydroxy-carboxylic acids, is then repeatedly washed with small quantities of water, which may be caused to rise to the top or settle to the bottom by appropriate control of the conditions. The wash water is found to contain some water-soluble compounds, and therefore preferably is transferred to the acid water tank 21 for the subsequent working up of values contained therein.

The water-free hydroxy-carboxylic acids are transferred from the separating tank 12, through the valved conduit 13, into the still 17 and are there subjected to a vacuum distillation treatment for the removal of substantially all of those components which would evaporate upon exposure of the product to the atmosphere over protracted periods of time. The specific conditions under which the distillation is conducted depend largely upon the desired physical character of the end product, but in general the operation should be conducted at a pressure of about 10-20 m. m. of mercury and at as low a temperature as possible for the substantially complete removal of volatilizable compounds,—e. g., from 140° to about 275° C. The relatively higher temperatures are required for the production of hard, brittle products, while lower temperatures, with correspondingly increased yields, are suitable for the production of relatively softer and less brittle products.

The volatilized material passing off from the still 17 under the influence of the partial vacuum maintained by the vacuum pump 20, and, preferably, assisted by a stream of air or steam admitted by the valved conduit 17, are condensed in condenser 18 and caught in having as one electrode a brass bar  $\frac{5}{8}$  inch

the distillate receiver 19. The latter distillate contains volatile, esterifiable acids of lower molecular weight which may be worked up for the recovery of values contained therein,—e. g., for the manufacture of esters,—and heavier carboxylic acids which may be returned to the oxidation cycle through the valved conduits 23 and 14' for conversion into hydroxy-carboxylic acids. It is noted that the carboxylic acids readily are converted into resin-like products, which characteristic apparently is due to the ease with which said acids polymerize.

The residue in the still 17, obtained by the carrying out of the above-described procedure, is the shellac-like product which is the basis of the invention. In general, it ranges in color from amber to dark brown; usually, the lighter the starting material (i. e., the unoxidized petroleum hydrocarbon mixture) the lighter the color of the end product. The product, apparently an acid, or acid anhydride body, is readily soluble in warm caustic soda solution or sodium carbonate solution, by which it is saponified to form soaps very similar to the soap produced by the saponification of natural shellac. It is insoluble in petroleum, in the fatty oils, and other similar oils, but is soluble in carbon tetrachloride. Depending upon the conditions maintained during the vacuum distillation operation, it ranges in consistency from a hard, brittle, readily grindable solid to a relatively softer, "tacky" product. The softer, "tacky" varieties are soluble in alcohol and in benzol, whereas the hard, brittle varieties are practically insoluble in those solvents.

The chief characteristic of this product, from an economic viewpoint, is its high dielectric property.

In order to arrive at a comparison of the relative dielectric properties of natural shellac and of the shellac-like product of the present invention, alcoholic solutions of the two substances were prepared by dissolving 55 grams of each in 67 grams of alcohol. Sheets of common writing paper, averaging 0.0033 inch in thickness, were coated or impregnated with the solutions and then allowed to dry for two days. Test pieces, each being of four thicknesses of the impregnated and dried paper were prepared and their relative thicknesses in inches ascertained to be:

Test piece using natural shellac..... { 0.0414 0.0418 0.0458 120  
0.0412 0.0382

Test piece using synthetic shellac..... { 0.040 0.039 0.039  
0.0388 0.0386

i. e., an average thickness of 0.0417 inch in the case of the test pieces using natural shellac, and 0.0391 inch in the case of the test pieces using synthetic shellac.

The dielectric capacities of these test pieces were ascertained on a test transformer

125  
130

in diameter and pointed at the end adjacent the test piece. At the same time the results were checked against the dielectric capacity of four-thickness test pieces built up of the uncoated or unimpregnated paper.

5 The following values were obtained:

*Dielectric capacity, measured in kilovolts*

|    | Test pieces using the synthetic shellac of the present invention | 8.0 | 8.2 | 8.2 | 8.0 | 8.0  | 8.15 | 8.6 |
|----|------------------------------------------------------------------|-----|-----|-----|-----|------|------|-----|
|    |                                                                  | 8.5 | 8.5 | 8.5 | 7.0 | 8.0  |      |     |
|    |                                                                  | 8.9 | 9.0 | 9.0 |     |      |      |     |
| 10 | Test pieces using natural shellac                                | 7.2 | 7.3 | 7.8 | 7.3 | 8.0  |      | 7.5 |
|    |                                                                  | 7.2 | 7.8 | 7.3 | 7.2 | 7.46 | 8.2  |     |
|    |                                                                  | 8.6 | 8.2 | 8.2 |     |      |      |     |
|    | Unimpregnated paper test pieces                                  | 3.8 | 3.0 | 3.3 | 3.3 | 3.0  | 3.3  |     |
|    |                                                                  | 3.2 | 3.0 | 3.2 | 2.8 |      |      |     |
|    |                                                                  | 2.9 | 2.7 | 2.9 |     |      |      |     |

15 It should be noted that the test pieces using the synthetic shellac, although somewhat thinner in cross-section than those using natural shellac, were found to have a higher dielectric capacity than the latter.

20 The tests demonstrated the fact that the synthetic shellac,—although "stickier" than the natural product,—has a higher melting point than that of natural shellac.

The above tests are summarized as follows:

| 25 | Average single thickness of paper used in test | Average thickness of test piece of paper impregnated with: |                     | Kilovolts dielectric capacity of unimpregnated paper—average of 13 trials | Kilovolts dielectric capacity of test piece comprising natural shellac—average of 15 trials | Kilovolts dielectric capacity of test piece comprising applicant's product—average of 16 trials |
|----|------------------------------------------------|------------------------------------------------------------|---------------------|---------------------------------------------------------------------------|---------------------------------------------------------------------------------------------|-------------------------------------------------------------------------------------------------|
|    |                                                | Natural shellac                                            | Applicant's product |                                                                           |                                                                                             |                                                                                                 |
|    |                                                | Inch 0.0033                                                | Inch 0.0417         |                                                                           |                                                                                             |                                                                                                 |
| 30 |                                                | 0.0391                                                     |                     | K <sub>v</sub> . 3.354                                                    | K <sub>v</sub> . 7.687                                                                      | K <sub>v</sub> . 8.37                                                                           |

35 The shellac-like product above described is adaptable for use in all insulation applications in which shellac is used. For example, it may be admixed with wood flour, asbestos, mica, wood pulp, or other inert materials in the same manner, and in about the same proportions in which shellac is used, for the production, under conditions of high temperature and pressure, of molded insulation, artificial lumber, and molded products generally.

40 For example, about 10 parts by weight of the hard, brittle shellac-like product are finely ground and thoroughly mixed with about 90 parts by weight of wood flour, and the mixture subjected to the same conditions of temperature and pressure as those customarily employed for the production of a composition molded insulation containing shellac. The resulting molded composition which is hard, dense and homogeneous, may be sawed, nailed, turned and generally worked in the same manner as a natural hard wood.

45 In substantially the same manner, there may be prepared molded articles containing 75-85% of asbestos, 85-70% of mica, or 50% of wood pulp admixed with said shellac-like product. In molded compositions such as those just mentioned, as well as in the com-

position forming the subject matter of the above example involving the use of wood flour, I have found that the shellac-like product advantageously may be used in the form of a salt,—as, for example, the calcium salt,—of the petroleum-insoluble hydroxy-carboxylic acids, in which form the product readily may be ground and admixed with the inert materials.

50 Also, it may be introduced, in finely divided condition, into paper pulp in the beating engine, for the production of a stiff, hard paper having high dielectric properties. In the form of a sticky, highly viscous product it may be used for the impregnation of tape for electric insulation, producing thereby a highly dielectric "tacky" tape which sticks well to the wire or to itself.

55 The shellac-like product, hereinbefore described, may be dissolved in suitable solvents to the production of a solution adaptable for use as a substitute for the commonly used solutions of natural shellac.

60 It is noted that the hard, brittle, shellac-like product above described may be prepared by merely exposing the petroleum-insoluble, saponifiable hydroxy-carboxylic acids, as obtained by the separation operation in separating tank 12, in thin films to a current of air at room temperature or thereabouts. However, such procedure is uneconomical in view of the fact that the valuable volatilizable compounds contained in the intermediate product thereby are lost.

65 While in the foregoing description the production of my shellac-like product has been described by reference to a batch process, it is to be understood that the invention is not restricted thereto, and that the process of making said product might well be carried out by recourse to a continuous or cyclic procedure, involving the controlled oxidation of a moving body of oil, continuous separation of the petroleum-insoluble hydroxy-carboxylic acids from the reaction mixture, and continuous return of unoxidized oil and partial oxidation products to the oxidizer.

70 While the production of the hereinbefore described shellac-like product is not restricted to any particular theory of oxidation reactions, the following is advanced as being a probable explanation of said reactions:

75 In regard to the reactions which may take place during the controlled oxidation of petroleum hydrocarbon mixtures by means of air under pressure at reacting temperatures, it is thought that the main primary reaction is one in which the oxygen attaches itself to a secondary carbon atom in the hydrocarbon chain and, in general, it is believed that the first secondary carbon atom after the primary carbon atom,—in other words the carbon atom in the  $\beta$ —position to the  $\text{CH}_3$  group at the end of any chain or branch,—is the one to which the oxygen first attaches itself. It

is the opinion, from many observations, that the oxygen is absorbed without the loss of any hydrogen; in other words, a hydroxyl group is formed at this point, thus forming a secondary alcohol.

- 5 The principal reason for assuming that this is the case is the fact that with the oxidation of a given mass of petroleum there is obtained as high as 15% of formic acid and it is believed that this is due to the end hydrocarbon radical being eliminated in the form of formic acid by the oxidation of a ketone formed from the secondary alcohol in which the hydroxyl is attached to the  $\beta$  carbon atom. The above conclusion is supported by the fact that when a secondary alcohol is oxidized it first forms a ketone. When a ketone which is a "methyl X ketone"—that is, one in which the methyl group is on one side of the CO group and a group of very much higher molecular weight is on the other side of the CO group,—such ketone oxidizes in such manner as to leave the CO group attached to the larger molecule, the CO group thus becoming the carboxylic group of the high molecular weight acids and the  $\text{CH}_3$  group forming formic acid. The rule in other words is that when ketones are oxidized the CO group attaches itself to the radical of higher molecular weight and the group of lower molecular weight is oxidized to the corresponding acid containing only the total number of carbon atoms which that group has minus the CO group.
- 35 This view is further supported by the fact that of the oil remaining after removal of all easily volatile and all acid products the greater proportion forms crystalline compounds with bisulphite, indicating the presence of rather large amounts of ketones or aldehydes but, as before stated, the opinion inclines to the formation of ketones rather than aldehydes because of the very large production of formic acid. When it is considered that one is treating hydrocarbons with an average composition around  $\text{C}_{20}\text{H}_{42}$  and that one obtains as high as 15% of actual formic acid there seems to be almost no other explanation for the main or principal reaction. It has been found also that the mixture of acids produced under conditions tending to avoid production of hydroxy-acids shows a molecular weight which, in most cases, corresponds to hydrocarbons of about 55% higher molecular weight than those chosen for the oxidation. This may be accounted for in two possible ways. There may be incipient oxidation in the end hydrocarbons,—that is, of the methyl group of the hydrocarbons,—in such a way as to effect what is known as the Kolbe reaction. If simultaneously, by an atom of oxygen, two hydrocarbon molecules are so oxidized that the methyl group, in the case of each molecule, loses one hydrogen atom, one would

have a synthesis immediately of the two hydrocarbon molecules forming one of twice the molecular weight less two hydrogen atoms. The other possible explanation, which would appear to be the stronger, is as follows: The acids when first formed are extremely liable to further oxidation and as in practically all cases one would have at the other end of a straight chain, or at any other branch, a carbon atom in relatively the same position as the first secondary carbon atom which had been oxidized to ketone and acid which also would be oxidized, probably almost simultaneously, to an alcohol. The acid in one case would either form a lactone with itself or would form an ester with the alcohol at the other end of the same chain in another molecule of the same or other acid, thus forming an ester-acid and, as the acids of lower molecular weight are frequently much more active in ester formation than those of higher molecular weight, it is probable that there would be a synthesis of this kind producing an average molecular weight of about 50% higher value than the simple acid theory would account for.

It seems proper to infer, from the above theory, that the oxidation reactions occur in such manner that very large molecules are formed by the esterification of hydroxy-acids by acids of the same, or higher, or lower, molecular weight, thus forming almost endless chains. Separations by partial precipitation have obtained from acids which show an average molecular weight of about 360, acids having molecular weights as high as 800 and, from the same mixture, there have been precipitated acids having molecular weights as low as 100. This is particularly true where the oxidation has been carried far enough to form petroleum-insoluble hydroxy-carboxylic acids. This would very naturally be the case since it is just these acids which we know are the hydroxy-acids as they show a considerable absorption of acetyl and we have now proof of their polymerization either through esterization or through polymerization due to the fact that they have the hydroxy group. This hydroxy group also may readily become a ketone group, as is readily perceivable. Ketones in themselves are also extremely active; especially, the higher ketones show a great tendency to polymerize. This may be an added cause for the production of acids of extremely high molecular weight.

An additional fact which supports the idea of ester acids or ketone acids being formed is that, if these higher molecular weight acids are distilled without too much destruction, there are obtained mixtures of lower molecular weight acids and ketones with some small quantities of hydrocarbons. The principal amount of material, however, comprises acids of lower molecular weight than those put in the still and ketones of not very high

molecular weight. This would appear to support the ester acids hypothesis.

This application is a division of my co-pending application Serial No. 156,052, filed Dec. 20, 1926.

5 I claim:

1. A molded article comprising inert filler and a material comprising saponifiable, water-insoluble, petroleum-insoluble hydroxy-carboxylic acids obtained by contacting a free-oxygen containing gas with a petroleum hydrocarbon mixture in liquid state at a reactive temperature of from about 100° C. to about 155° C., and at a pressure greater than atmospheric, producing thereby saponifiable, water-insoluble, petroleum-insoluble hydroxy-carboxylic acids, separating the said acids from the reaction mixture, and subjecting the separated acids to vacuum distillation.

10 2. A molded article comprising about 90 parts by weight of wood flour and about 10 parts by weight of a material comprising saponifiable, water-insoluble, petroleum-insoluble hydroxy-carboxylic acids obtained by contacting a free-oxygen containing gas with a petroleum hydrocarbon mixture in liquid state at a reactive temperature of from about 100° C. to about 155° C. and at a pressure greater than atmospheric, producing thereby saponifiable, water-insoluble, petroleum-insoluble hydroxy-carboxylic acids, separating the said acids from the reaction mixture and subjecting the separated acids to vacuum distillation.

15 35 In testimony whereof, I affix my signature.  
ARTHUR W. BURWELL.

40

45

50

55

60

65